

N. S. Clements.

Table Cutlery.

N<sup>o</sup> 88,544.

Patented Mar. 6, 1869.



Witnesses,  
C. A. Shepard  
Wm. G. Coutts

Inventor.  
Nathan S. Clement.  
By James Shepard Atty



NATHAN S. CLEMENT, OF NEW BRITAIN, CONNECTICUT.

*Letters Patent No. 88,544, dated April 6, 1869.*

**IMPROVEMENT IN CASTING HANDLES OF TABLE-CUTLERY.**

The Schedule referred to in these Letters Patent and making part of the same.

*To all whom it may concern:*

Be it known that I, NATHAN S. CLEMENT, of New Britain, in the county of Hartford, and State of Connecticut, have invented a new and useful Improvement in Table-Cutlery; and I do hereby declare that the following is a full, clear, and exact description thereof, which will enable those skilled in the art to make and use the same, reference being had to the accompanying drawings, making a part of this specification, in which—

Figure 1 is a side elevation of my invention.

Figure 2 is a longitudinal section of the same, drawn through the line *x-y*.

Similar letters of reference indicate like parts.

My invention consists of casting the handles of table-cutlery, of cast-iron or steel, hollow, by means of a core, one end of which is supported by a print in the sand, or mould, in the usual manner, and the other end is supported by the tang of the cutlery-blade to be handled.

To cast these handles, a pattern is first made, of the shape of the body of the handle *c* and bolster, which bolster is formed on, and is a part of the handle *c*. On one end of the handle-pattern is formed a small projection, to form a core-print in the sand. In the other, or bolster-end of the handle *c*, I insert the tang *b*, of the cutlery-blade *a*, designed to be handled, with the said blade *a* in its proper position.

A print, or mould of the pattern and blade *a* is then made in the usual manner, and the pattern and blade withdrawn from the sand. The tang *b*, of the blade *a*, is then inserted a short distance into one end of the core, when the blade *a* and core are placed in the print from which the blade and pattern have been withdrawn, with the core supported at one end in the print formed by the projection on the end of the handle-pattern, while the tang *b*, which is inserted in the other end of the core, will hold it in its place.

The core should be short enough to leave a portion of the tang *b* exposed, which portion of the tang *b* can be nicked, or serrated, if desired. The mould is then ready to close, and the iron or steel poured into it in the usual manner. The metal will form a shell around

the core, and the bolster-end of the handle *c* will form solid around the tang *b*, filling the serrated portions, and thus securing the handle *c* firmly to the blade *a*. The whole is then taken from the sand, and the core removed through the open end *e* of the handle *c*.

A small cap, *d*, is then brazed, or soldered, or otherwise secured to the open end *e* of the handle *c*, when the handle is ready to polish and finish.

If desired, a false tang, or a tang-shaped implement might be used to support one end of the core in casting, and then withdrawn, when the tang proper can be secured by a subsequent process.

Handles have been formerly cast of white-metal, or metals that fuse at a low heat, but such metals are also softer, and consequently easily bruise, and become soiled.

Handles have also been formed in two halves, either swaged of wrought-metal, or cast of alloys, and then soldered together.

Others have been cast in metallic moulds, after the usual manner of casting hollow ware of soft metal, *viz*, when the outer portion of the metal is chilled, pour out the interior.

It is also common to cast the bolster around the tang, after the handle has been formed and secured to the blade, and sometimes the bolster is cast first, and the handle afterward secured.

By my invention, I am able to secure the advantages of hardness, durability, and other qualities of handles cast from metal which require a high temperature to fuse, forming them with the requisite lightness and great cheapness of production.

I do not claim, broadly, casting hollow handles, unless by the means of the metal described; neither do I claim casting the bolster around the tang, or bolsters or handles formed of wrought-metal; but

What I claim as new, and desire to secure by Letters Patent, is—

Casting the handles of table-cutlery hollow, by the process herein specified.

NATHAN S. CLEMENT.

Witnesses:

JAMES SHEPARD,  
Wm. G. CURTISS.